

## UNITED STATES PATENT OFFICE.

ARTHUR S. O'NEIL, OF ALTON, ILLINOIS, ASSIGNOR TO WESTERN CARTRIDGE COMPANY, OF EAST ALTON, ILLINOIS, A CORPORATION OF DELAWARE.

PROPELLANT POWDER AND PROCESS OF MAKING SAME.

No Drawing.

Application filed September 4, 1923. Serial No. 660,939.

This invention relates to propellant powders, and more particularly to nitro-cellulose powders adapted for use in and suitable for smooth-bore guns and small arms.

- 5 In my copending application, Serial Number 618,388, is described a process for modifying the surface of a dense colloided nitro-cellulose powder grain so that it will approach the rate of burning of the so-called 10 bulk powders, and in order that this rate of burning may be so accelerated that the initial pressure is developed at the rate required to enable its utilization in and render it suitable for cylinder guns and small arms.
- 15 In accordance with the process described, a dense colloided nitro-cellulose powder grain, (such as military ammunition salvaged from the war, sub-divided to the required extent) is modified so as to form a 20 dense core surrounded by a less dense and porous envelope. This is accomplished by swelling the surface of the grain to the desired depth of penetration and the swollen envelope so formed is then fixed. This fixing is accomplished in such a manner as to 25 cause not only interruption of the swelling in order to secure an envelope of the desired depth, but also to break up the surface in order to leave an open and porous envelope 30 which is readily ignitable.

One of the objects of this invention, therefore, is to further improve the propellant powder and process.

Another object of this invention is to provide a propellant powder in which the dense colloided nitro-cellulose grain is impregnated with an oxidizer.

Another object of this invention is to improve the sub-division of the powder grain 40 in order to obtain a flaky grain having improved characteristics.

Further objects will appear from the detail description in which is given an example illustrating a practical embodiment of this 45 invention. In this illustration we will assume as a base material a dense colloided nitro-cellulose powder, such as standard untreated military ammunition salvaged from

the war, although the process is equally applicable to freshly prepared nitro-cellulose 50 powders, or even surface treated powders.

In accordance with this invention the powder is reduced to the form of flakes; these flakes are, however, irregular and in fact warped. This reduction can be accomplished in any suitable manner so as to secure the desired result. A suitable process comprises in reducing the grains in a beater such as is used for pulping gun cotton. Such a beater has an anvil or stationary cutter with which cooperates a series of knives on a drum, and these are immersed and operate in an annular tank which can be filled with water, which water is adapted to circulate in and along the tank and past the 55 cooperating faces of the anvil and knives. The action is to slice the powder grains so as to form flakes, that is, grains whose widths and lengths are much greater than their thicknesses. By the cooperation of the 60 knives on the drum with the anvil or stationary cutter, the flakes while being formed by slicing the grains, are, however, squeezed or compressed so as to reduce the grain thickness. Moreover these flakes will be uneven and 65 warped. The presence of the water not only prevents ignition but also promotes the formation of flaky grains. The reduction of the powder grains to flake form may, however, be performed in other ways, as by 70 passing the grains between two burrs or discs rotating face to face and provided with radial teeth, which have a slicing as well as a flattening action, in that they serve to flatten out the cut or broken grain in the form 75 of flakes. Furthermore the grains may be flattened by passing the same through heavy calender rolls, and these flakes may then be further reduced by grinding in any suitable manner. In each case, however, the operations are performed in the presence of water. After flaking, the grains may be dried and screened to remove any dust, and the screening may be performed to proper sizes for 80 different calibers or arms.

There is thus produced a powder grain 85 90 95

which is in the form of a thin flake. A grain of this description has certain desirable characteristics not found in other shapes, and in the case of a powder for use in smooth-bore guns, has the distinct advantage of producing a semi-progressive propellant. Bulk powder for example burns very rapidly and produces high breech pressures, and powders of the highly progressive type, 5 while lower in breech pressure, are apt to throw undue pressures along the barrel and thus cause ruptures in the gun. The flake powder owing to its shape and method of production eliminates these objectionable 10 features and produces a powder which burns in the proper manner to produce the highest ballistic efficiency. The uneven or warped character of the flake also has the advantage over a plain flat grain in that two uneven or 15 warped grains cannot lie flat against one another; accordingly the burning of each flake can proceed uniformly, thereby avoiding irregular ballistics.

The powder so reduced may be used to advantage in smooth-bore guns without further treatment. It is, however, preferably given the further treatment described in the application referred to. Furthermore the 20 hereinafter described treatment may be applied to a powder not of the flake form. A practical example of this treatment will now be described.

Taking again, for illustration, as a base a dense colloided nitro-cellulose powder, this 25 is sub-divided or reduced to the required state of divisions to form grains either of the flaky form or otherwise. This powder is then intimately mixed with a solid nitro-hydrocarbon, such as dinitro-toluene, in the 30 proportion of ninety-eight (98) parts of the powder and two (2) parts of the solvent, although the proportions may be varied within limits to suit requirements. The mixture is then introduced into a tank provided with 35 a stirring mechanism, or into a tumbling barrel, which tank or barrel has been previously filled with water and raised to a temperature of 75° to 100° C., depending upon the nature of the solvent used. The 40 temperature is maintained (by supplying live steam or water to a jacket or by the direct action of steam) for a suitable period, in case where dinitro-toluene is used for a period of about 1/2 hour, while the powder 45 and the solid solvent are rumbled together in the solution. The solvent under the influence of heat melts and distributes itself uniformly over the powder grain, and due to its solvent action penetrates the same, with 50 the result that there is formed an envelope of nitro-cellulose collidized with dinitro-toluene, which is less dense than the body or core of the grain. Cold water is now admitted to the mixture so as to rather suddenly chill the contents of the barrel, there-

by causing the dinitro-toluene to lose its solvent properties and partially recrystallize, while a portion of the nitro-cellulose together with a part of the solvent is also partially precipitated from the colloid, so that the 55 envelope will become partially decolloided. The result is, therefore, a powder grain having a dense colloided nitro-cellulose core and a cracked and porous envelope, and the grain as a whole has become of greater volume. 75

The treatment as just described is fully described in application Serial No. 618,388 referred to, to which reference is had for further detail description. In accordance with the present invention, however, the 80 powder grain is impregnated with an oxidizer, such as a suitable metallic nitrate, of which barium nitrate, potassium nitrate and sodium nitrate are examples. These salts readily enter the porous envelope when applied in the form of a solution, which solution enters the pores or cracks; upon drying the salt remains behind in the envelope as an integral part of the powder grain.

As a practical illustration of a practical 85 embodiment of this invention, the nitrate salt is added to the water during the application of the dinitro-toluene, since it will not interfere with the action of the solvent. Accordingly the heating and chilling steps are 90 performed in the presence of this salt solution acting as a heating medium, and this solution enters the pores and cracks of the grain envelope. When now the grains so treated are removed from the solution and dried in the usual manner, the envelope will not contract but will remain porous due to the chilling step, while upon evaporation of the water from the salt solution in the pores, this salt will remain behind in the pores. 100 The quantity of oxidizer introduced into the powder grain depends largely upon the strength of the solution, and its strength need not be fixed since the solution may be reused again and again. However, as a practical example a five percent solution will give satisfactory results. 105

It will, therefore, be seen that a powder grain is formed which has a core of dense colloided nitro-cellulose and a porous envelope impregnated with an oxidizer. The structure of the envelope is, therefore, such that it is not only readily ignitable, but it will continue to burn at a higher rate under a reduced pressure, so that the burning of 110 the envelope supplies the necessary temperature and pressure to afford complete combustion of the balance of the grain. This rate of combustion can be regulated by variation of the thickness of the envelope, which can readily be controlled by extending the penetration period of the solvent. Moreover the impregnation of the grain with the oxidizer 115 will produce a grain which contains sufficient oxygen for complete combustion; accordingly 120 125 130

the weight of the charge is reduced to obtain equal ballistics. While the impregnation of a grain may be applied to dense colloided nitro-cellulose powders generally, it is of especial advantage when applied to the uneven or flaky grains as heretofore described, since this renders the resultant powder particularly advantageous for use in smooth-bore or shot guns.

10. It will be understood that the above detail description is of an illustrated embodiment of this invention, and that the same may be varied in various ways without departing from the spirit of this invention.

15. Thus the impregnation of the powder grains with the salt may be accomplished after the grain has been acted upon by the solvent and chilled; thus the powder may, after the action of the solvent thereon and after the 20 same has been fixed by chilling, be taken from the tank or tumbling barrel and dumped into a tank or vat containing the salt solution, and after penetration for a suitable period, the powder may be removed 25 from the solution and dried. It is further obvious that various changes may be made in details without departing from the spirit of this invention; it is, therefore, to be understood that this invention is not to be limited to the specific details shown and described.

Having thus described the invention, what is claimed is:

1. A propellant powder grain of dense colloided nitro-cellulose the surface layer only of which is impregnated with an oxidizer.
2. A propellant powder grain of dense colloided nitro-cellulose the surface layer only of which is impregnated with a metallic 40 nitrate.
3. A propellant powder grain of dense colloided nitro-cellulose the surface of which is porous and has an oxidizer within and filling the pores.
4. A propellant powder grain comprising, a dense colloided nitro-cellulose core surrounded by a porous envelope impregnated with an oxidizer.
5. A propellant powder grain of dense colloided nitro-cellulose the surface of which is partially decolloided and impregnated with an oxidizer.
6. A propellant powder grain of dense colloided nitro-cellulose the surface layer only of which is colloided with a solvent and impregnated with an oxidizer.
7. A propellant powder grain of dense colloided nitro-cellulose the surface of which contains a precipitated nitro-hydrocarbon and a metallic nitrate.
8. In the art of making propellant powder, the process comprising, rendering the surface of the grain porous and impregnating the surface with an oxidizer.
9. In the art of making propellant powder,

the process comprising, swelling the surface of the grain and impregnating the surface with an oxidizer.

10. In the art of making propellant powder, the process comprising, swelling the 70 surface of the grain, impregnating the surface with an oxidizer, and fixing the envelope so formed.

11. The process comprising, subjecting a dense nitro-cellulose colloid to the action of 75 a swelling medium and impregnating the envelope so formed with an oxidizer.

12. The process comprising, subjecting a dense nitro-cellulose colloid to the action of a solvent and an oxidizer in order to impregnate the surface layer only thereof.

13. The process comprising, subjecting a dense nitro-cellulose colloid to the action of a solvent, chilling the envelope so formed, and impregnating the envelope with an oxi- 85 dizer.

14. The process comprising, heating a dense nitro-cellulose colloid with a solid nitro-hydrocarbon solvent and impregnating the envelope so formed with a metallic ni- 90 trate.

15. The process comprising, heating a dense nitro-cellulose colloid with a solid nitro-hydrocarbon in a water solution of a metallic nitrate.

16. The process comprising, heating a dense nitro-cellulose colloid with a solid nitro-hydrocarbon in a water solution of a metallic nitrate and chilling the same in such solution.

17. The process comprising, reducing dense colloided nitro-cellulose powder grains in the presence of water so as to form flakes.

18. The process comprising, grinding dense colloided nitro-cellulose powder grains 105 in the presence of water into flakes.

19. The process comprising, reducing dense colloided nitro-cellulose powder grains and forming the same into flakes.

20. The process comprising, breaking 110 dense colloided nitro-cellulose powder grains and flattening the same to form flakes.

21. The process comprising, slicing dense colloided nitro-cellulose powder grains so as to form flakes.

22. The process comprising, slicing dense colloided nitro-cellulose powder grains and reducing the thickness of the same.

23. A broken propellant powder grain of dense colloided nitro-cellulose in the form of 120 a flake.

24. A propellant powder grain of dense colloided nitro-cellulose in the form of an irregular flake.

25. A propellant powder grain of dense 125 colloided nitro-cellulose in the form of a warped flake.

26. A propellant powder grain of dense colloided nitro-cellulose in the form of a flake the surface of which is porous.

27. A propellant powder grain of dense colloided nitro-cellulose in the form of a flake the surface of which is impregnated with an oxidizer.
28. A propellant powder grain of dense colloided nitro-cellulose in the form of a flake the surface of which is partially de-colloided.
29. A propellant powder grain of dense colloided nitro-cellulose in the form of a flake the surface of which is partially de-colloided and impregnated with an oxidizer.

In testimony whereof I affix my signature this 22nd day of August, 1923.

ARTHUR S. O'NEIL.